

# United States Patent [19]

Katz

[11] 3,820,919

[45] June 28, 1974

[54] ZIRCONIUM-CARBON GETTER MEMBER

[75] Inventor: Helmut Katz, Munich, Germany

[73] Assignee: Siemens Aktiengesellschaft, Berlin, Munich, Germany

[22] Filed: Dec. 13, 1971

[21] Appl. No.: 207,022

## [30] Foreign Application Priority Data

Dec. 21, 1970 Germany..... 2062992

[52] U.S. Cl..... 417/48, 252/181.6

[51] Int. Cl..... F04b 37/00

[58] Field of Search..... 252/181.6; 313/174, 176, 313/178; 417/48, 49, 51

## [56] References Cited

### UNITED STATES PATENTS

|           |         |               |           |
|-----------|---------|---------------|-----------|
| 1,733,809 | 10/1929 | Lederer ..... | 417/51 X  |
| 2,043,724 | 6/1936  | Anderson..... | 417/48    |
| 2,167,852 | 8/1939  | Rose .....    | 417/48    |
| 2,175,695 | 10/1939 | Kniepen.....  | 252/181.6 |
| 2,208,692 | 7/1940  | Wamsley.....  | 417/48    |

|           |         |                  |           |
|-----------|---------|------------------|-----------|
| 2,824,640 | 2/1958  | Della Porta..... | 417/48    |
| 2,855,368 | 10/1958 | Perdijk.....     | 252/181.6 |
| 3,102,633 | 9/1963  | Baronetzky ..... | 417/51    |
| 3,225,910 | 12/1965 | Della Porta..... | 417/48    |
| 3,428,168 | 2/1969  | Reash .....      | 417/51    |
| 3,560,788 | 2/1971  | Reash .....      | 417/51    |
| 3,584,253 | 6/1971  | Wintzer .....    | 417/51    |

Primary Examiner—William L. Freeh  
Attorney, Agent, or Firm—Hill, Gross, Simpson, Van Santen, Steadman, Chiara & Simpson

## [57] ABSTRACT

A getter member comprised of an open-ended container composed for example of molybdenum or carbon, having a sintered porous mass composed of a mixture of zirconium and up to about 30 percent by weight carbon therein. The getter member is non-evaporable and operable at room temperatures so as to be positionable at any desired location within an electric discharge tube. Means for securing the getter material within its container is also disclosed.

1 Claim, 9 Drawing Figures



PATENTED JUN 28 1974

3,820,919



Fig. 7



Fig. 8



Fig. 9



INVENTOR

Helmut Katz

BY

Lill, Sherman, Meroni, Gross & Simpson

ATTYS.

## ZIRCONIUM-CARBON GETTER MEMBER

## BACKGROUND OF THE INVENTION

## 1. Field of the Invention

The invention relates to getters and more particularly to getter members operable at room temperatures in electric discharge tubes.

## 2. Prior Art

It is known to completely enclose vaporizable getter materials within a container and position the same within an electric discharge tube so that a getter material mirror-like film is produced on the envelope of the tube, as by HF annealing. A serious drawback with such vaporizable getter materials is that it is difficult to control the getter material vapors and it is extremely important to avoid depositing getter material film on any important parts of a discharge tube, particularly on any insulating parts thereof.

Such drawbacks are substantially eliminated with non-evaporating getter materials, however, non-evaporating getter materials must be heated, either temporarily, repeatedly or continuously, within the discharge tube by special heating devices thereby rendering such getters uneconomical.

The invention provides non-evaporating getter members that substantially eliminate the prior art drawbacks.

## SUMMARY OF THE INVENTION

The invention provides non-evaporating getter members comprised of substantially open-ended container of molybdenum or carbon having a porous sintered getter material therein comprised of a mixture of zirconium and up to about 30 percent carbon. The getter members of the invention are operable at room temperatures and are attached to a desired position of an electric discharge tube without heating devices. The adhesion between the container and the getter material is sufficiently great so that as a general matter, no special securing is required to insure retention of the getter material within the container. However, with particularly valuable tubes, such securing is reassuring. Accordingly, certain embodiments of the invention include means of securing the getter material within the container, such as wires, cap-like structures, shaped bars or similar members attached to the container and holding the getter material therein. The securing means can be attached to the container and sintered in with the getter material or be attached after the getter material has been sintered.

## BRIEF DESCRIPTION OF THE DRAWINGS

FIG. 1 is an elevated sectional view of an embodiment constructed in accordance with the principles of the invention;

FIG. 2 is a somewhat similar view of another embodiment of the invention;

FIG. 3 is also a similar view of yet another embodiment of the invention;

FIG. 4 is a similar view of a further embodiment of the invention;

FIG. 5 is a partial elevated sectional view of another embodiment of the invention;

FIG. 6 is a view somewhat similar to FIG. 5 of a further embodiment of the invention;

FIG. 7 is an elevated sectional view of a further embodiment of the invention;

FIG. 8 is a somewhat similar view of a modified form of the invention illustrated at FIG. 7; and

FIG. 9 is a partial elevated sectional view of another embodiment of the invention.

## DESCRIPTION OF THE PREFERRED EMBODIMENTS

10 The invention provides getter members operable at room temperatures in electric discharge tubes or the like wherein the getter material is positioned within a substantially open-ended container, for example, in an open-ended recess of a sheet-metal container that is

15 readily securable to operating portions or to other portions of an electric discharge tube. The non-evaporating getter material of the invention is comprised of a mixture of zirconium and up to about 30 percent by weight carbon (graphite) sintered into a

20 highly porous mass. The container is composed of relatively high temperature resistant material, such as molybdenum or carbon and is attachable at a desired position within an electric discharge tube. Heating devices are not necessary for the getter members of the invention.

25 The adhesion between the container and the getter material mass is of a sufficient strength so that generally no securing means therebetween is required. However, when the getter member of the invention is utilized in a particularly valuable discharge tube, various types of securing means are provided to prevent the getter material mass from falling out of the container.

30 The securing means include wires, sheet-caps, rods, Z-shaped or U-shaped bars as well as other similar structures generally composed of molybdenum, tantalum or other similar metals. The securing means are attached to the container by various means, such as spot-welding, crimping, passing through portions thereof, etc., and are attached to the getter material by being embedded therein or by contacting a surface portion thereof. The securing means are attached to the getter material either prior to the sintering process and sintered in with the getter material or are suitably attached after the sintering process.

35 The invention results from systematic investigations with zirconium-carbon mixtures conventionally applied to arrangements that are adapted for periodic, repeated or continuous heating, for example, as applied to a heating coil insulated with aluminum oxide. It was discovered that a large getter capacity can be obtained from such a mixture without heating. The zirconium-carbon mixtures have getter characteristics, particularly when in a large pore sintered state, that are suited for production of getter members operable at room temperatures. Such getter members are heated only once during the production of a particular discharge tube and are thereby freed of their own gases to such a degree that they have a sufficiently large capacity for additional gases, even in a cold state over extended periods of time.

40 The range of composition of the zirconium-carbon mixture is relatively broad and varies from about a minimum of 70 percent by weight of zirconium and a maximum of about 30 percent carbon. The maximum amount of zirconium in the mixture is about 90 to 95 percent while the minimum amount of carbon in the

mixture is about 5 to 10 percent. Accordingly, a preferred way of expressing the composition of this mixture is to indicate that it is comprised of a mixture of about 70 percent to 95 percent by weight of zirconium and about 5 percent to 30 percent by weight of carbon.

The getter material of the invention have particularly good adhesive characteristics to the material of the container as well as to itself so that no loose particles are present. Accordingly, a getter mass formed from such materials can be utilized as a relatively thick layer. The getter members of the invention having such relatively thick layers of getter material have a gas capacity, which even in a cold state exceeds the gas capacity of presently known getters.

Referring now to the drawings, wherein like reference numerals referred to like elements, FIG. 1 illustrates a getter member embodiment comprised of a container 1 composed for example of molybdenum, formed into an open-ended body having an interior recess or the like. A sintered mass 2 composed of a mixture of zirconium and carbon is positioned and tightly bonded to the interior recess of the container 1.

FIG. 2 illustrates a somewhat modified form of the getter member embodiment discussed in FIG. 1, wherein one or more molybdenum wires 3 are spot-welded onto the exterior portions of the container 1 so as to prevent the sintered mass 2 from falling out.

In a further modified form shown at FIG. 3, a molybdenum Z-shaped bar is spot-welded to the bottom of the interior recess of container 1 and then embedded in the zirconium-carbon mixture and sintered in with the mass 2 so as to secure the same from displacement.

FIG. 4 illustrates a further modified embodiment of a getter member wherein a tantalum sheet or strip 5 is crimped onto the exterior flanges of the container 1 and extends over at least a portion of the opening thereof for maintaining the mass 2 in position.

FIGS. 5 and 6 illustrate cylindrical getter member embodiments wherein a sheet-metal container 11, for example, formed of a high-temperature resistant material such as molybdenum or carbon, is filled with a zirconium-carbon mixture sintered into a highly porous mass 12. In order to insure that the mass 12 does not become detached from its container, securing means are provided. In FIG. 5, such securing means comprise a bent wall portion 14 of the container 11, while in FIG. 6, the securing means comprise a wire 13 attached to the interior of container 11 and embedded within the mass 12.

The embodiments illustrated at FIGS. 7, 8 and 9 are comprised of a substantially open-ended carbon con-

tainer 21, filled with a sintered mass 22 of a zirconium-carbon mixture. The adhesion between the carbon container 21 and the mass 22 is extremely good and very reliable during operation. Accordingly, the embodiment illustrated at FIG. 7 does not utilize any special securing means. In the embodiment illustrated at FIG. 8, a rod 23, as of molybdenum penetrates through opposing wall portions of the container 21 and through the mass 22 to insure that the mass 22 does not become detached from the container. In the partial view of the embodiment shown in FIG. 9, a U-shaped member 24 is inserted and penetrates through opposed wall portions of container 21 and through mass 22 so as to secure the same from displacement.

During production of the getter members of the invention a recess is formed, for example, in a thin molybdenum sheet by the application of suitable pressure. The formed recess is substantially completely filled with a suitably formulated viscous zirconium-carbon mixture, as by smearing. The getter member is then sintered. It is then ready for insertion into a discharge tube, even a relatively small tube. During production of discharge tubes, they are heated, for example, by high frequency (HF) and the getter material is freed of gas. In another embodiment, a relatively small tube or cylinder, for example of molybdenum, of a given diameter is formed and filled with a zirconium-carbon mixture. The so-filled tube is then sintered and suitably attached in a discharge tube. In embodiments wherein the getter members are of relatively large dimensions, it is useful in at least certain instances to provide securing means to insure that the getter material does not separate from its container, as in the form of a zirconium-carbon plug or the like.

Various changes and modifications to the above described embodiments of the invention may be made without departing from the spirit and scope thereof and is intended that all matters contained in the above description shall be interpreted as illustrative and not as limiting.

I claim as my invention:

1. A getter member for operating at room temperature in an electric discharge tube comprised of a container having a substantially open-ended recess therein, said container being composed of a relatively high-temperature resistant material selected from the group consisting of molybdenum and carbon, and a sintered porous non-evaporable gettering mass attached within said recess, said sintered porous gettering mass being comprised of a mixture of about 70 to 95 percent by weight of zirconium and about 5 to 30 percent by weight of carbon.

\* \* \* \* \*